

## UNITED STATES PATENT OFFICE

2,145,746

ANODE FOR ELECTRODEPOSITION OF  
TUNGSTEN

Harry Howard Armstrong and Arthur Burley  
Menefee, Beverly Hills, Calif., assignors to  
Tungsten Electrodeposit Corporation, Wash-  
ington, D. C., a corporation of Delaware

No Drawing. Application May 18, 1935,  
Serial No. 22,281

12 Claims. (Cl. 204—4)

This invention relates to the electrodeposition of metals, more particularly to the production and use of special types of anodes peculiarly useful for the electrodeposition of metals, such as tungsten and alloys thereof.

The present invention is in part a continuation of our prior applications Serial No. 744,566, filed January 5, 1935, and Serial No. 14,372, filed April 2, 1935.

0 As disclosed in the prior applications above referred to, we have found that adherent, dense, fine grained and acid resistant plates of tungsten with variable percentages of other metals may be electrodeposited from suitable aqueous baths.

5 As there explained, under very wide permissive limits of hydrogen ion concentration, dilution, current density and so forth, tungsten alloys or alloys of metals similar to tungsten may be deposited from aqueous fluoride baths. We have further found, as explained in the designated applications, that the tungsten ions may be made available in the bath either by dissolving tungsten compounds directly in a suitable aqueous solution of a fluoride or by subjecting a tungsten 10 containing electrode to anodic corrosion in a fluoride bath.

We have now found that a relatively wide variety of specifically different tungsten containing compounds may be employed as the main anode 0 for the electrolytic cell or as, so-to-speak, replenishing anodes, whereby an effective concentration of tungsten ions and/or other metal ions may be maintained in the bath.

An object of the invention, therefore, is to provide novel types of electrodes, particularly useful for the electrodeposition of tungsten or similar metals and alloys thereof.

Another object is to provide a tungsten containing electrode of satisfactory electrical conductivity.

5 A further object is to provide a novel composite electrode for electrodepositing two or more metals.

A still further object is to utilize as a tungsten ion producing agent an electrode composed of a tungsten compound of high conductivity and ready availability.

Yet another object is to provide an electrode for 0 the electrodeposition of tungsten comprising a compound of tungsten and a non-metal of high conductivity.

A further object is to provide an electrode for use in the electrodeposition of tungsten alloys 5 comprised of a tungsten containing compound in

intimate association with a second metal or metals.

With these and other equally important and related objects in view the invention comprehends the concept of producing special electrodes for 5 effective employment in the electrodeposition of tungsten and alloys thereof.

The electrodes of the present invention, it is to be clearly understood, are employable either in the process described in prior application Serial 10 No. 744,566 or Serial No. 14,372, that is to say either in an electrolytic bath in which all of the tungsten ions are produced by electrolysis of a tungsten metal compound or in an electrolyte in which tungsten ions are initially made available by direct dissolution of a tungsten compound 15 in a suitable solvent, such as a bi-fluoride, and the tungsten concentration maintained by continuous or intermittent electrolysis of a tungsten metal compound.

As explained in prior application Serial No. 744,566 eminently satisfactory plates may be secured by first establishing a hot definitely acid aqueous bath containing an acid fluoride, such as sodium acid fluoride and an agent, such as sodium chloride, which imparts high conductivity to the bath, and then electrolyzing using a tungsten containing anode, such as tungsten carbide or a tungsten alloy carbide. The electrolysis preferably is carried out under conditions of high 20 acid concentration, of the order of pH 4 more or less. Upon satisfactory electrolysis the hydrogen ion concentration is then preferably adjusted to a lower value and the desired basis metal or cathode is then plated. Tungsten carbide and tungsten 25 alloy carbides serve effectively for such a process. Such massive materials present a satisfactory electrical conductivity and effective corrosion of the metal content.

In further experimentation we have found that 40 a number of specifically different types of anodes may be employed. Some of these are particularly useful in special adaptations of the process. Thus we have found that under properly controlled conditions, particularly of current density 45 and temperature, the respective amounts of the constituent metals of the ultimate alloy may widely be varied during a given plating operation. In such a process it is desirable to have available a rapidly or readily corrodible quantity of a second metal or metals to be coplated with tungsten to form the final alloy. In these circumstances, as will be appreciated, it is advantageous to utilize main anodes or replenishing anodes which present a large area for wetting or contact by the 50

electrolyte to thus accelerate the corrosion of the desired metal and provide a higher metal concentration in the bath. For the same reason in some circumstances it is desirable to make the second metal or metals available in the relatively pure and unassociated form, thus further accelerating the corrosion rate of this metal.

It will thus be seen that by providing a wide range of anodes of specifically different composition and character the plating process may be made much more flexible and the ramifications of use of the ultimate plate considerably widened. According to one phase of the invention, therefore, the tungsten supplying material may comprise substantially pure tungsten. This may consist of discrete tungsten metal packed or tamped in an acid proof anode container. Again the tungsten powder may be compressed under relatively high pressure and fitted as a core in a conductive acid proof anode. The relatively pure tungsten may likewise be made available either as the main anode or a replenishing or regenerating electrode by admixing tungsten powder with a suitable bonding or cementing agent, preferably of a carbonaceous character, and subjecting the mass to heat and/or pressure to form a compact rugged electrode. Similarly tungsten powder may be compacted and cemented under heat and pressure to form an electrode of suitable strength and relatively large exposed area.

Such electrodes may be employed alone or in conjunction with inert or reactive anodes to carry out plating operations as described in the prior applications referred to.

It will be appreciated also that in making up each of the anodes above described there may be added suitable quantities of other powdered metals, such as nickel, chromium, cobalt, iron, cadmium, antimony and the like, when electrodeposited alloys of tungsten and one or more of such metals are desired.

Because of its adequate tungsten content, satisfactory conductivity and ready availability, tungsten carbide provides a good anode material for employment in the present process. Heretofore operations have been carried out utilizing massive tungsten carbide. We have found that tungsten carbide powder when compacted, or when cemented either with suitable cementing materials, or directly cemented under heat and pressure, likewise serves very effectively. Like tungsten metal powder, this may be employed in relatively loose condition in a suitable acid proof anode container or be made up in the compacted self-sustaining form. Similarly predetermined percentages of relatively discrete or packed and/or cemented mixtures of tungsten metal and tungsten carbide powder may be utilized. A wide range of relatively standardized anodes for plating different types of alloys may be fabricated by homogeneously incorporating in the tungsten carbide mass or in the tungsten metal-tungsten carbide units, predetermined amounts of other coplatable metals, such as nickel, cobalt, antimony, chromium and the like.

As has been fully described in the prior applications, one of the striking characteristics of these several fluoride baths defined therein is the capability of directly dissolving not only tungsten oxides, such as  $WO_2$  and  $WO_3$ , but also the tungstates meta and para tungstates. Thus, as explained in application Serial No. 14,372, satisfactory electrodeposition of tungsten alloys may be secured by directly dissolving, say a tungstic acid anhydride in hot ammonium bifluoride. Upon

addition of other desirable adjuvants, such as sodium fluoride, boric acid, tartaric acid and a soluble salt of the second metal or metals to be alloyed with tungsten, an alloy plate may be procured when using an inert anode or an anode of a metal other than tungsten.

This characteristic of the new electrolyte permits the use of special forms of anodes and by such use achieves improved results. Thus an anode may be made up which comprises a predominant quantity of tungsten containing compound, such as compacted tungsten metal powder, tungsten carbide powder or a mixture of tungsten metal powder and tungsten carbide powder, together with a minor percentage of a soluble tungsten compound, such as tungsten dioxide or tungsten trioxide. It will be appreciated by those skilled in the art that the quantity of the soluble tungsten compound may be so chosen that it will leach or dissolve out of the anode without materially impairing the structural strength of the anode. In these circumstances, therefore, the tungsten ion concentration of the bath may be maintained by supplying tungsten not only by means of anodic corrosion of a conductive tungsten compound but also by slow dissolution of a soluble tungsten compound. Since the soluble tungsten compound is uniformly distributed throughout the anode, it is thus made available at a slow and relatively constant rate. It likewise will be appreciated that in the bath of the character described, during electrolysis a relatively high concentration of hydrofluoric acid obtains at the anode, thus facilitating the dissolution of the tungsten oxide impacted in the massive anode.

This type of anode may be made up as hereinbefore described. For example a predetermined quantity of tungsten metal powder may be homogeneously admixed with a minor quantity of a soluble tungsten compound and then compacted under suitable conditions of temperature and pressure or the mass may be cemented by a suitable binder. A similar procedure may be employed in making up an anode comprising a mixture of predetermined major quantities of tungsten metal powder and tungsten carbide powder and a minor quantity of the soluble tungsten compound. As described above, anodes may be made up containing the tungsten powder, tungsten carbide powder, or a combination of the two in admixture with tungsten oxides or other soluble tungsten compound and containing in addition to these predetermined quantities of powdered or discrete metals which are to be coplated with the tungsten for the production of an electrodeposited alloy. It is particularly to be observed that when tungsten metal is to be employed for the anode, complete reduction need not be effected; that is to say when utilizing a bath of the characteristics defined herein, it is possible to use tungsten metal containing a small percentage of tungsten oxide. Thus when the tungsten metal which is employed as the anode is made by reduction from the oxides, a complete reduction is not essential; hence cheaper forms of relatively pure tungsten metal may be employed effectively in the present invention.

What has been said of the employment of tungsten metal and tungsten carbide applies similarly to tungsten alloys. Suitable commercial tungsten alloys may be utilized as anode materials in the present invention. Again it will be understood that, if desired, the anode employed may itself be an electrodeposited alloy plate. Thus, for example, it is within the con-

cept of the invention to provide anodes by plating out tungsten and other metals, such as nickel, in the form of an alloy on a typical cathode. For this use the plate does not have to be as adherent or fine-grained as the ultimate plate and hence operative conditions may be so controlled as to secure the maximum amount of plated metal. Such alloy surface may be electrodeposited upon a basis metal or, and preferably, upon a carbon core. Such alloys may be in the massive form or in the discrete or powdered form when suitably treated to provide a compact self-sustain electrode. Such materials likewise may be used in the relatively uncompacted form by utilizing an acid resistant anode container for the material.

While preferred modifications of the invention have been described, it is to be understood that these are given merely as examples of the underlying principles involved and not as definitive of the exclusive methods of effectuating such principles. It will be appreciated that within the scope of the concepts herein expressed, other and specifically different but equivalent electrodes may be fabricated which function in an analogous manner. All such modifications or extensions as are included within the scope of the appended claims are considered to be comprehended within the spirit of the invention.

30 We claim:

1. An electrode for use in the electrodeposition of tungsten which comprises a compacted mixture of discrete tungsten metal and tungsten carbide.
2. An electrode for use in the electrodeposition of tungsten which comprises an intimate compacted mixture of tungsten metal and an oxide of tungsten.
3. An electrode for use in the electrodeposition of tungsten which comprises an intimate compacted mixture of tungsten carbide and an oxide of tungsten.
4. An electrode for use in the electrodeposition of tungsten which comprises an intimate coin-

pacted mixture of discrete tungsten metal, tungsten carbide and an oxide of tungsten.

5. An electrode unit for use in the electrodeposition of tungsten which comprises an intimate mixture of discrete tungsten metal, tungsten carbide and a cementing agent. 5

6. An anode for use in the electrodeposition of alloys of tungsten which comprises a compacted mixture of discrete tungsten metal and nickel. 16

7. An anode for use in the electrodeposition of alloys of tungsten which comprises a compacted mixture of discrete tungsten carbide and nickel.

8. An anode for use in the electrodeposition of alloys of tungsten which comprises a compacted 15 mixture of discrete tungsten metal, tungsten carbide and nickel.

9. An anode for use in the electrodeposition of alloys of tungsten which comprises a compacted mixture of discrete tungsten metal and 20 a second metal coplatable with tungsten and comprised within the group consisting of nickel, chromium, cobalt, iron, cadmium, and antimony.

10. An anode for use in the electrodeposition of alloys of tungsten which comprises a compacted mixture of discrete tungsten carbide and 25 a second metal coplatable with tungsten and comprised within the group consisting of nickel, chromium, cobalt, iron, cadmium, and antimony.

11. An anode for use in the electrodeposition 30 of alloys of tungsten which comprises a compacted mixture of discrete tungsten metal, tungsten carbide, and a second metal coplatable with tungsten and comprised within the group consisting of nickel, chromium, cobalt, iron, cad- 35 mium, and antimony.

12. An anode unit for use in the electrodeposition of alloys of tungsten which comprises a uniform mixture of tungsten carbide and discrete metals coplatable with tungsten and comprised within the group consisting of nickel, 40 chromium, cobalt, iron, cadmium, and antimony.

HARRY HOWARD ARMSTRONG.

ARTHUR BURLEY MENESEE.